

# United States Patent Office

3,479,163

Patented Nov. 18, 1969

1

3.479.163

3,475,163

**STABILIZATION OF PETROLEUM DISTILLATE  
FUELS BY OXIDATIVE TREATMENT**

Elliot A. Vogelfanger, Edison, and Thomas J. Wallace,  
Elizabeth, N.J., assignors to Esso Research and Engi-  
neering Company, a corporation of Delaware  
No Drawing. Filed Jan. 3, 1966, Ser. No. 518,033  
Int. Cl. C10I 1/10; B01j 1/16

12 Claims

U.S. Cl. 44—64 12 Claims

## 12 Claims

## **ABSTRACT OF THE DISCLOSURE**

Solids free petroleum distillate fuels which are resistant to further atmospheric oxidation are obtained by treating petroleum distillate fuels which originally contained olefinic unsaturated components and molecular oxygen, i.e., air, with at least one metallocene and at least one aryl hydrazone followed by the removal of at least the resultant solid gum formed thereby by any suitable means such as settling, decantation, centrifugation, filtration and/or distillation.

The present invention relates to the stabilization of petroleum distillate fuels containing olefinic unsaturated components through an oxidative treatment. In particular, it relates to the stabilization of fuels having boiling ranges within the boiling range of between about 75° F. and about 750° F. whereby it is possible to improve the stability of such fuels by oxidative degradation and to thus greatly alleviate the gum-forming tendencies of such fuels when stored or standing under atmospheric conditions and in contact with the atmosphere, which atmosphere contains molecular oxygen.

The petroleum industry has long recognized the instability of distillate petroleum fuels, boiling between about 75° F. and about 750° F. or having boiling ranges within this range, largely due to the presence of olefinic unsaturated components in such fuels. This constitutes a serious problem in connection with the use, handling, and storage of the fuels because of the unstable constituents, chief among which are the mono and diolefinic components, tend to gradually oxidize or otherwise react. For example, polymerization or copolymerization occurs during storage to form gums, sludges, and/or sediments which either precipitate out of the fuel or which remain in solution in the fuel and are later deposited through vaporization or combustion of the fuels in fuel lines, carburetors, pistons, cylinder walls and other surfaces in internal combustion engines thus causing breakdown in lubrication and a general gumming up in internal combustion engines. Such clogging and deposition of either precipitate or dissolved gums or sludge which have formed as a result of the co-oxidation or oxidation of the olefinic components necessitates the disassembling of the engine and the cleaning of all moving parts including carburetors fuel lines, filters and the like. This becomes an extremely expensive operation and entails time consuming effort. In the past, this has sometimes been controlled to some extent through the addition of antioxidants to the petroleum distillate fuels containing the olefinic components.

In a copending application, Ser. No. 517,908 filed Jan. 3, 1966 by Thomas J. Wallace and Norman Friedman entitled "Oxidative Treatment of Petroleum Distillate Fuels Containing Olefinic Unsaturated Components," a new and improved method of treating such unsaturated petroleum distillates, in order to accelerate the formation of gum and sludge through polymerization and/or co-polymerization of the olefinic components thereof, there is disclosed a use of certain arylhydrazones. It is shown therein that once the major portion of the readily oxidiz-

2

able and polymerizable olefinic components are removed as polymers, either soluble or insoluble in nature, the resultant distillate fuel is stabilized against further atmospheric oxidative degradation to a large extent. In that application it is directed to add between about 0.1 and about 1% by weight, preferably between about 0.3 wt. percent and about 0.6 wt. percent of one or more specific arylhydrazones in the presence of molecular oxygen, i.e., air, which may either be dissolved in the fuels or in contact with the fuels during such treatment. Neither the time of contact nor the temperature is important in such treatment but it is preferred to use a temperature of from atmospheric up to about 150° F. for a sufficient time of contact of the arylhydrazones with the olefinic feedstocks to allow for substantial oxidative polymerization or copolymerization of the olefinic constituents thereof. The time of contact may range anywhere from between about 30 minutes up to several hours, for example, up to 8 to 50 hours or even longer. The length of time is generally that amount of time during which substantial quantities of oxygen are consumed or taken up in the reaction. It has subsequently been discovered that this may last up to 172 to 200 hours where atmospheric temperatures are employed.

25 Following the treatment the solid or existent gums  
are removed by settling, decantation, centrifugation, or  
filtration. A subsequent atmospheric or vacuum distilla-  
tion, if convenient, will result in an overhead distillate  
30 or condensate substantially free of potential or soluble  
gum, the residue containing such gum. Fuels so treated  
are effectively stabilized against any substantial oxidative  
reactions and so they remain stable over prolonged  
periods of time and during actual use. If desired, they  
35 may be stabilized against further oxidation by the use  
of conventional antioxidants as additives thereto. Such  
antioxidants, for example, are: 2,6-di-tertiary butyl  
phenol, para-amino phenol, di-phenylamine, and N,N'-  
40 di-secondary - butyl-para-phenylenediamine. Convention-  
ally these are added in amounts up to about 0.01 wt.  
percent and thus effect stabilized fuels which remain so  
over long periods of time of the order of many weeks  
or months.

The arylhydrazones employed are those having the formula:



wherein R may be a C<sub>1</sub>–C<sub>12</sub> saturated acyclic hydrocarbon radical such as methyl, ethyl, isopropyl, propyl, butyl, isobutyl, octyl, iso-octyl, dodecyl and the like or may further be a C<sub>5</sub>–C<sub>12</sub> saturated cyclic aliphatic hydrocarbon radical such as cyclopentyl, cyclohexyl, cycloheptyl and the like, an aralkyl radical such as benzyl, phenethyl or an aryl radical such as phenyl, naphthyl or anthryl. R' may be the same as or different from R as above defined, R and R' may be jointly a C<sub>4</sub>–C<sub>5</sub> alkylene (cycloaliphatic) radical or R' may be hydrogen. It has been discovered, however, that R<sub>1</sub> may not be an aryl radical if R is also an aryl radical. The arylhydrazine reacted with this ketonic or aldehydic compound must be an arylhydrazine such as phenylhydrazine, naphthylhydrazine, or anthrylhydrazine. Representative hydrazones employed are the phenylhydrazones of cyclohexanone, cyclopentanone, benzylaldehyde, para-tolyl aldehyde, dibenzyl ketone, acetophenone, 9-anthraldehyde, 1-naphthaldehyde, and 2-naphthaldehyde. The arylhydrazones may be formed by reacting the hydrazine with a mixed ketoaldehyde such as pivalyl aldehyde, a dialdehyde such as phthaldehyde, or a diketone such as cyclohexanedione or cyclopentanedione. As used in this description and

accompanying claims, the definitions of R and R<sub>1</sub> are intended to encompass the mixed ketoaldehydes, the diketones, and the dialdehydes.

It has now been discovered that improved rates of oxidation with resultant polymerization and copolymerization can be accomplished and improved amounts of existent and potential gums formed if there is used, in conjunction with the hydrazones mentioned above, an effective amount of one or more metallocenes. The amount of the metallocene may vary considerably but, in general, the distillate fuel being treated will contain an arylhydrazone to metallocene weight ratio of between about 1:1 and about 10:1, preferably between about 3:1 and about 6:1. Larger amounts of metallocenes may be employed with regard to the amount of arylhydrazones used but, because of the cost of the metallocenes, the rate of oxidation, and the total amount of polymerization or copolymerization of the olefinic constituents is not sufficiently increased to warrant the extra expense of using the larger amounts of metallocenes; the total amount of mixed treating agent used (hydrazone+metallocene) is preferably between about 0.1 and about 7.0 wt. percent, preferably between about 0.4 and about 0.7 wt. percent. The two types of additives may be premixed and added to the fuel or either one may be first added and the other one subsequently added.

The metallocenes are formed through the interaction of Group VIII metal inorganic salts with cyclo olefins or their simple methyl and ethyl derivatives. Any metal of Group VIII of the Periodic System, according to Mendeleeff, may constitute the metal portion of the metallocene. Specific examples of suitable metal components of the metallocene are: iron, cobalt, nickel, ruthenium, osmium, and the like. The olefinic portion of the metallocene is preferably derived from cyclopentadiene although other cyclo olefins such as cyclo-octadiene, cyclo-octatetraene, cyclo-butadiene and benzene, for example, are also suitable as reactants. Any of the conventional methods for the preparation of the metallocenes may be employed, for example, ferrocene may be produced by reacting ferric or ferrous chloride in ethyl ether with a solution of cyclopentadienyl magnesium bromide or ferrous chloride may be reacted with cyclopentadiene under nitrogen at 300° F. in the presence of alumina, molybdena, or the like in the presence of potassium oxide. U.S. Patents 2,680,756 and 2,791,597 disclose representative methods of preparing the metallocenes. The use of ammonium salts or of alkali metal salts of cyclopentadiene in liquid ammonia followed by the addition of anhydrous metal nitrate or phthalocyanate, the metal being a Group VIII metal, results in a complex which loses ammonia on heating, in vacuum, to give the corresponding metallocene. The present invention is not concerned with any particular method of preparing the metallocenes, any of the methods heretofore known being suitable for their production.

Representative metallocenes which are useful as additives, when used in conjunction with the aforementioned arylhydrazones, are the following: cyclopentadienyl iron (ferrocene), cyclopentadienyl nickel (nickelocene), cyclopentadienyl cobalt (cobaltocene), cyclopentadienyl ruthenium (ruthenocene), cyclopentadienyl osmium (osmocene); acylmetallocenes such as acetylferrocene, formylferrocene, benzoylferrocene, benzoylruthenocene, arylmetallocenes such as phenylferrocene, 1,3,1',3'-tetraphenylferrocene, p-ferrocenylphenol, p-ferrocenylaniline, dibenzoruthenocene; and the alkyl-substituted cyclopentadienyl metallocenes such as methylferrocene, 1,1'-diisopropylferrocene, and 1,1'-trimethyleneferrocene. The metallocenes and their method of preparation are fully disclosed in Rosenblum "Chemistry of the Iron Group Metallocenes," a volume in the series The Chemistry of Organometallic Compounds, published by Interscience Publishers, a division of John Wiley & Sons (1965), which reference work is incorporated hereinto by reference.

The oxidative treatment of the petroleum distillate fuels containing olefinic unsaturated components involv-

ing the combined use of arylhydrazones and metallocenes, as above described and defined, applies to a wide range of gasolines and heating oils. These may be derived from gas oils of any desired boiling range through the conventional steam cracking, thermal cracking, or catalytic cracking of the same. Almost any cracked naphtha or heating oil contains considerable quantities of olefinic compounds. These olefinic compounds, depending upon the particular process by which the feed was produced, can be either cyclic or acyclic in nature. They can be mono-olefinic or di-olefinic (either conjugated, nonconjugated, or of the allenic type). In some cases polymeric forms of olefins are present in the cracked naphthas as produced, generally in soluble form. Any of the cyclic or acyclic olefinic unsaturated compounds such as indene, or even styrene, will be effectively polymerized or copolymerized through the novel arylhydrazone treatment herein described. Typical olefins found in cracked naphthas and heating oils include the following: 2-hexene, cyclohexene, indene, 1,3-hexadiene, 1-pentene and 4-methyl-2-hexene. Any number of these olefinically unsaturated compounds other than those specifically mentioned tend to render gasoline or heating oils unstable during storage.

Additionally, and depending upon the source of the crude oil which has been used, these distillate fuels may also contain nitrogen compounds such as pyrroles, indoles, aliphatic amines and pyridines; disulfides; and finally mercaptans of both aliphatic and aromatic nature. Although it is not intended that the instant novel process be limited by any theory, it is believed that substantial portions of these types of impurities also undergo oxidative reaction involving polymerization and/or oxidative reaction involving copolymerization of those impurities with some of the olefinic components present and so are likewise converted into gums or sludges which can be removed in the same manner and at the same time as the gums and sludges formed solely from the olefinic constituents.

The presence of other additives in the treated distillates such as antiknock agents, scavenging agents, dyes, anti-icing agents, and solvent oils in total additive concentration not exceeding 5% by wt. does not adversely affect the oxidative treatment with arylhydrazones and metallocenes for the purpose of forming gums. Conversely, the treatment with arylhydrazones and metallocenes does not adversely affect the functioning of the aforementioned conventional additives for their intended purpose, so that it is possible to successfully carry out the oxidative gum formation operation on either finished or unfinished gasolines or heating oils, which contain the olefinic components.

Representative specific types of naphthas and heating oils to which the invention applies are heavy catalytic naphthas, light catalytic naphthas, No. 2 heating oil, and the like. Typical and representative chemical and physical inspections of two such naphthas are as follows:

|                                                     | Heavy<br>Catalytic<br>Naphtha | Light<br>Catalytic<br>Naphtha |
|-----------------------------------------------------|-------------------------------|-------------------------------|
| 60 Gravity, ° A.P.I.                                | 25                            | 57.9                          |
| Initial Boiling Point, ° F.                         | 430                           | 77                            |
| Final Boiling Point, ° F.                           | 650                           | 430                           |
| Research Octane Number                              | 55                            |                               |
| Wt. percent aromatics                               | 47.1                          | 11.3                          |
| Wt. percent mono olefins-diolefins (cyclic+acyclic) | 26.3                          | 57.8                          |
| 65 Wt. percent saturates (cyclic+acyclic)           | 26.6                          | 30.9                          |

#### Example 1

A heavy catalytically cracked naphtha of the type above stated in 200 cc. aliquots, except as otherwise noted, was treated with about 1 wt. percent of three different phenylhydrazones alone or in conjunction with one or more metallocenes present in an amount of about 0.1 wt. percent. For purposes of these percentages in this example and the following examples, 200 cc. of naphtha

feed or regular gasoline is considered to weigh 200 grams. All operations were carried out at 25° C. which is considered to be atmospheric temperature. The results and conditions of treatment are shown in Table I. The first run shown is a blank run involving no treatment with either a phenylhydrazone or a metallocene and is shown for comparative purposes only. The comparative tests were carried out as follows:

A 500 cc., round bottom, 4-necked flask was equipped

than 72 hours had been left standing for one or more days with oxygen in contact therewith so that, to some extent, they were already partially oxidized and, to some extent, had partially lost their oxidizing activity. In any case, the times of contact are those times deemed to have been necessary to secure substantially complete consumption of oxygen using the particular reactants and under the particular conditions obtaining at the time.

The data in Table I clearly point out the advantage of

TABLE I.—HEAVY CATALYTIC NAPHTHA FEED (200 cc.)

| Oxidative Reagent                       | Amount in grams (weight percent) | Time of Contact (hours) | Treat. Temp. (° C.) | Total gum (mg./100 cc. of feed) |                     |
|-----------------------------------------|----------------------------------|-------------------------|---------------------|---------------------------------|---------------------|
|                                         |                                  |                         |                     | Existent (Solid)                | Potential (Soluble) |
| Blank                                   |                                  |                         | 25                  | 34                              | 844                 |
| Cyclohexanone phenylhydrazone (250 cc.) | 2.5(1.0)                         | 24                      | 25                  | 605                             | 1,584               |
| (Fresh) Cyclohexanone phenylhydrazone   | 2.0(1.0)                         | 119                     | 25                  | 977                             | 2,221               |
| Plus Ferrocene                          | 0.2(0.1)                         | 72                      | 25                  | 932                             | 2,321               |
| Plus Nickelocene                        | 0.2(0.1)                         | 72                      | 25                  | 1,402                           | 2,403               |
| Plus Cobaltocene                        | 0.2(0.1)                         | 72                      | 25                  | 1,212                           | 4,794               |
| Acetophenone phenylhydrazone            | 2.0(1.0)                         | 71                      | 25                  | 370                             | 2,820               |
| Plus Nickelocene                        | 0.2(0.1)                         | 72                      | 25                  | 1,378                           | 2,728               |
| Plus Cobaltocene                        | 0.2(0.1)                         | 72                      | 25                  | 1,756                           | 3,694               |
| Cyclopentanone phenylhydrazone          | 2.0(1.0)                         | 69                      | 25                  | 273                             | 1,041               |
| (Fresh) Cyclopentanone phenylhydrazone  | 2.0(1.0)                         | 171                     | 25                  | 547                             | 1,505               |
| Plus Cobaltocene                        | 0.2(0.1)                         | 72                      | 25                  | 2,607                           | 4,030               |

with a paddle stirrer, an overhead water-cooled condenser, a thermometer, and a self-sealing rubber cap. Molecular oxygen was supplied to the vessel from a partially filled polyethylene gas balloon, through a wet-test gas meter through which oxygen was passed, connected to a drying tower packed with a desiccating material such as Drierite (anhydrous magnesium sulfate). There was then introduced into the reaction vessel through the neck of the flask 200 to 250 cc. of naphtha and 2 to 2.5 grams of the particular phenylhydrazone and metallocene, when used. The system was then purged with oxygen, sealed with the rubber cap, and the wet-test meter adjusted to zero volume when an equilibrium pressure was established. The reaction was then started by rapid stirring and was allowed to proceed until no further oxygen consumption could be detected on the wet-test meter. All experiments were conducted at atmospheric pressure.

In the following tables, the column headed "Existent (Solid)" and the column headed "Potential (Soluble)" added together give the total gum formed in the treating process; the existent gum being precipitated from the naphtha and recovered by filtration and weighed in terms of milligrams per 100 cubic centimeters of naphtha and the potential gum being soluble gum which was recovered after distilling to dryness and weighing the gum. These figures are also in terms of milligrams of gum per 100 cc. of feed.

using small amounts of metallocene in conjunction with the phenylhydrazones to increase both existent and potential gum content. For example, the existent gum of the heavy catalytic naphtha is increased from 34 to 977 mg./100 cc. feed (about 30-fold) by adding about one weight percent cyclohexanone phenylhydrazone. When a small amount (about 0.1 wt. percent) of nickelocene is employed together with the same phenyl hydrazone, the existent gum is increased by about 45-fold to 1402 mg./100 cc. of feed. Similarly cobaltocene in conjunction with cyclopentanone phenylhydrazone increases the existent gum number of the heavy catalytic naphtha by about 76-fold to 2607 mg./100 cc. of feed. Significant increases in potential gum content were also obtained by the addition of small amounts of the same metallocenes in combination with the same phenylhydrazones as seen by a comparison of the data in the extreme right-hand column of Table I.

#### Example 2

In a manner similar to that described in Example 1, a light catalytic naphtha having the inspection above stated was treated with two specific cyclo olefinic phenylhydrazones with and without admixture with various metallocenes as shown in Table II. The time conditions and the oxidative reagent employed, the amount of solid and soluble gums formed and the like are shown in Table II.

TABLE II.—LIGHT CATALYTIC NAPHTHA FEED (200 cc.)

| Oxidative Reagent              | Amount in grams (weight percent) | Time of Contact (hours) | Treat. Temp. (° C.) | Total gum (mg./100 cc. of feed) |                     |
|--------------------------------|----------------------------------|-------------------------|---------------------|---------------------------------|---------------------|
|                                |                                  |                         |                     | Existent (Solid)                | Potential (Soluble) |
| Blank                          |                                  |                         | 25                  | 6.6                             | 308                 |
| Cyclohexanone phenylhydrazone  | 2.0(1.0)                         | 71                      | 25                  | 560                             | 1,361               |
| Plus Ferrocene                 | 0.2(0.1)                         | 72                      | 25                  | 870                             | 1,256               |
| Plus Nickelocene               | 0.2(0.1)                         | 72                      | 25                  | 624                             | 955                 |
| Plus Cobaltocene               | 0.2(0.1)                         | 72                      | 25                  | 641                             | 3,552               |
| Cyclopentanone phenylhydrazone | 2.0(1.0)                         | 72                      | 25                  | 420                             | 817                 |
| Plus Nickelocene               | 0.2(0.1)                         | 72                      | 25                  | 754                             | 1,983               |
| Plus Cobaltocene               | 0.2(0.1)                         | 72                      | 25                  | 1,004                           | 1,117               |

In this example as well as the following examples, with respect to the tables, the designation "fresh" with respect to cyclohexanone phenylhydrazone or cyclopentanone phenylhydrazone is intended to differentiate a distinction as to time of use as between those hydrazones and the same hydrazone used in some cases for comparative purposes which was not "fresh" at the time of usage. In other words, those runs employing 72 hours for time of contact employed freshly prepared cycloaliphatic phenylhydrazone, whereas, those not so designated and where the time of contact may be either shorter or longer

Again, as in Example 1, appreciable increases in existent and potential gum content were obtained by the use of small quantities of metallocene with phenylhydrazones in the light catalytic naphtha. For example, while cyclohexanone phenylhydrazone alone increased the existent gum content to 560 mg./100 cc. feed, the admixture of 0.1 wt. percent ferrocene increased this number still further to 870 mg./100 cc. feed while, with neither additive being used, the gum content was 6.6 mg./100 cc. feed. The potential gum content of the light catalytic naphtha was also increased by more than 10-fold by the use of

a catalytic quantity of cobaltocene in conjunction with cyclohexanone phenylhydrazone. Similar results were also obtained from the cyclopentanone phenylhydrazone cobaltocene combination.

## Example 3

A regular, commercially available, catalytically cracked gasoline having a boiling range of 100° F.-350° F., a research octane number of 87, and a chemical composition of 45 wt. percent of cyclic+acyclic olefins and diolefins, 30 wt. percent of aromatics, and 25 wt. percent of paraffins and naphthenes was treated with cyclohexanone phenylhydrazone, benzaldehyde phenylhydrazone, and acetophenone phenylhydrazone; each alone and in combination with the various metallocenes as shown in Table III. The table also shows the total amount of existent and potential gums formed in each case.

TABLE III.—REGULAR GASOLINE (200 cc.)

| Oxidative Reagent                      | Amount<br>in grams<br>(weight<br>percent) | Time of<br>Contact<br>(hours) | Total gum (mg./100<br>cc. of feed) |                     |                        |
|----------------------------------------|-------------------------------------------|-------------------------------|------------------------------------|---------------------|------------------------|
|                                        |                                           |                               | Treat.<br>Temp.<br>(°C.)           | Existent<br>(Solid) | Potential<br>(Soluble) |
| Blank                                  |                                           | 24                            | 25                                 | 6.6                 | 3                      |
| Cyclohexanone phenylhydrazone:         |                                           |                               |                                    |                     |                        |
| 500 cc. of feed                        | 2.5 (0.5)                                 | 140                           | 25                                 | 333                 | 753                    |
| 500 cc. of feed                        | 0.5 (0.1)                                 | 51                            | 25                                 | 121                 | 766                    |
| (Fresh) Cyclohexanone phenylhydrazone: | 2.0 (1.0)                                 | 72                            | 25                                 | 720                 | 1,201                  |
| Plus Ferrocene                         | 0.2 (0.1)                                 | 72                            | 25                                 | 658                 | 1,024                  |
| Plus Nickelocene                       | 0.2 (0.1)                                 | 72                            | 25                                 | 615                 | 1,048                  |
| Plus Cobaltocene                       | 0.2 (0.1)                                 | 72                            | 25                                 | 867                 | 1,140                  |
| Benzaldehyde phenylhydrazone:          | 2.0 (1.0)                                 | 72                            | 25                                 | 549                 | 690                    |
| Plus Ferrocene                         | 0.2 (0.1)                                 | 72                            | 25                                 | 231                 | 891                    |
| Plus Nickelocene                       | 0.2 (0.1)                                 | 72                            | 25                                 | 862                 | 1,197                  |
| Plus Cobaltocene                       | 0.2 (0.1)                                 | 72                            | 25                                 | 624                 | 1,064                  |
| Acetophenone phenylhydrazone:          | 2.0 (1.0)                                 | 72                            | 25                                 | 329                 | 727                    |
| Plus Nickelocene                       | 0.2 (0.1)                                 | 72                            | 25                                 | 908                 | 1,422                  |
| Plus Cobaltocene                       | 0.2 (0.1)                                 | 72                            | 25                                 | 983                 | 1,479                  |

With regular gasoline, as was the case with light and heavy catalytic naphthas, distinct improvements in the gum content were obtained by the incorporation of small quantities of a metallocene with a phenylhydrazone. Specifically, with acetophenone phenylhydrazone as the 40 hydrazone and 0.1 wt. percent cobaltocene, the existent gum was increased to 983 mg./100 cc. feed from 6.6 mg./100 cc. feed (blank). This constitutes a 133-fold increase in the gum content. The amount of potential gum was also increased by a factor of four by the same phenylhydrazone-metallocene combination.

In the foregoing tables, the amount of hydrocarbon feedstocks used are shown in most instances to be 200 cc. aliquots and the additives are shown to be in terms of grams with the weight percent shown in parenthesis following the number of grams used. It is, of course, apparent that an accurate weight percent figure would be, in all cases, slightly higher than as shown because the volume of feed (200 cc.) would not weigh 200 grams but would actually vary between about 170 and about 185 grams depending upon the actual densities of the feedstocks employed.

Having now thus fully described and illustrated the instant novel process and compositions, what is desired to be secured by Letters Patent is:

1. A process which comprises treating, in the liquid phase, a petroleum distillate fuel containing olefinically unsaturated components and molecular oxygen with at least one metallocene and at least one arylhydrazone having the formula:



wherein R is selected from the group consisting of C<sub>1</sub>-C<sub>12</sub> saturated acyclic hydrocarbon radicals, C<sub>5</sub>-C<sub>12</sub> saturated cycloaliphatic radicals, aralkyl and aryl, R<sub>1</sub> is selected from the group consisting of C<sub>1</sub>-C<sub>12</sub> saturated acyclic hydrocarbon radicals, C<sub>5</sub>-C<sub>12</sub> saturated cycloaliphatic hydrocarbon radicals, aralkyl, and hydrogen, including R and R' being jointly a C<sub>4</sub>-C<sub>5</sub> alkylene radical, the weight ratio of arylhydrazone to metallocene being between about 1:1 and about 10:1, and from which so treated fuel at least the solid gum has been removed.

50  
55  
60  
65  
70  
75

and R' being jointly a C<sub>4</sub>-C<sub>5</sub> alkylene radical, the weight ratio of arylhydrazone to metallocene being between about 1:1 and about 10:1, and removing from the so treated distillate fuel at least the solid gum formed thereby.

2. A process as in claim 1 wherein the arylhydrazone used is the phenylhydrazone of cyclopentanone and the metallocene is selected from the group consisting of ferrocene, nickelocene and cobaltocene.

3. A process as in claim 1 wherein the arylhydrazone used is the phenylhydrazone of cyclohexanone and the metallocene is selected from the group consisting of ferrocene, nickelocene and cobaltocene.

4. A process as in claim 1 wherein the arylhydrazone used in the phenylhydrazone of acetophenone and the metallocene is selected from the group consisting of ferrocene, nickelocene, and cobaltocene.

5. A process as in claim 1 wherein the distillate fuel is a cracked naphtha boiling within the range between about 75° F. and about 750° F.

6. A process as in claim 5 wherein the arylhydrazone is obtained by reacting a cycloaliphatic saturated hydrocarbon ketone with phenylhydrazine.

7. A solids free petroleum distillate fuel originally containing olefinic unsaturated components and molecular oxygen which has been treated with at least one metallocene and at least one arylhydrazine having the formula:



wherein R is selected from the group consisting of C<sub>1</sub>-C<sub>12</sub> saturated acyclic hydrocarbon radicals, C<sub>5</sub>-C<sub>12</sub> saturated cycloaliphatic radicals, aralkyl and aryl, R<sub>1</sub> is selected from the group consisting of C<sub>1</sub>-C<sub>12</sub> saturated acyclic hydrocarbon radicals, C<sub>5</sub>-C<sub>12</sub> saturated cycloaliphatic hydrocarbon radicals, aralkyl, and hydrogen, including R and R' being jointly a C<sub>4</sub>-C<sub>5</sub> alkylene radical, the weight ratio of arylhydrazone to metallocene being between about 1:1 and about 10:1, and from which so treated fuel at least the solid gum has been removed.

8. A petroleum distillate fuel as in claim 7 wherein the arylhydrazone used is the phenylhydrazone of cyclopentanone and the metallocene is selected from the group consisting of ferrocene, nickelocene, and cobaltocene.

9. A petroleum distillate fuel as in claim 7 wherein the arylhydrazone used is the phenylhydrazone of cyclohexanone and the metallocene is selected from the group consisting of ferrocene, nickelocene, and cobaltocene.

10. A petroleum distillate fuel as in claim 7 wherein the arylhydrazone used is the phenylhydrazone of acetophenone and the metallocene is selected from the group consisting of ferrocene, nickelocene, and cobaltocene.

11. A petroleum distillate fuel as in claim 7 wherein

the distillate fuel is a cracked naphtha boiling within the range between about 75° F. and about 750° F.

12. A petroleum distillate fuel as in claim 11 wherein the arylhydrazone is obtained by reacting a cycloaliphatic saturated hydrocarbon ketone with phenylhydrazine.

3,088,960 5/1963 Wollensak.  
3,088,961 5/1963 Wilkinson.

## OTHER REFERENCES

Aurieth et al.: The Chemistry of Hydrazine, copyright 1951, John Wiley & Sons, Inc. pp. 226 and 227.

DANIEL E. WYMAN, Primary Examiner

Y. H. SMITH, Assistant Examiner

U.S. Cl. X.R.

252—400, 403, 186

## References Cited

## UNITED STATES PATENTS

|           |         |                  |         |    |
|-----------|---------|------------------|---------|----|
| 2,680,756 | 6/1954  | Pauson           | 252—431 | 10 |
| 2,680,758 | 6/1954  | Thomas           | 260—439 |    |
| 2,942,957 | 6/1960  | Wojcik           | 44—64   |    |
| 2,791,597 | 5/1957  | Anzilotti et al. | 44—68   |    |
| 3,064,020 | 11/1962 | Riemschneider    |         |    |